# EUROPEAN PATENT SPECIFICATION

(11) **EP 0 383 035 B1**
(45) Date of publication and mention of the grant of the patent: **04.10.1995**
(21) Application number: 90100930.8
(22) Date of filing: 17.01.1990
(51) Int. Cl.: H01F 1/20, H01F 1/26

(54) **Iron-silicon alloy powder magnetic cores and method of manufacturing the same**
Magnetkerne aus Eisen-Silizium-Legierungspulver und Herstellungsverfahren
Noyau magnétique en poudre d'alliage de fer-silicium et procédé de fabrication

(30) Priority: 18.01.1989 JP 7853/89; 25.12.1989 JP 335899/89
(43) Date of publication of application: 22.08.1990
(73) Proprietor: Nippon Steel Corporation, Chiyoda-ku Tokyo 100 (JP)
(72) Inventor: Nishida, Tokuhiko, c/o Nippon Steel Corporation, Kawasaki City, Kanagawa Prefecture (JP); Yamamiya, Masao, c/o Nippon Steel Corporation, Kawasaki City, Kanagawa Prefecture (JP)
(74) Representative: VOSSIUS & PARTNER

(56) References cited:
- EP-A- 0 087 781
- EP-A- 0 088 992
- EP-A- 0 135 980
- PATENT ABSTRACTS OF JAPAN vol. 9, no. 212 (E-339) 29 August 1985,& JP-A-60 074602 (NIHON FERRITE KK) 26 April 1985,
- PATENT ABSTRACTS OF JAPAN vol. 9, no. 212 (E-339) 29 August 1985,& JP-A-60 074603 (NIHON FERRITE KK) 26 April 1985,

## Description

This invention relates to a process of manufacturing iron-silicon alloy powder magnetic cores used in noise filters and choke coils for switching power supplies and powder cores obtainable by such process.

The prior art includes the following process for manufacturing materials for powder magnetic cores used in magnetic noise suppression and choke coils. Specifically, the process is as follows: magnetic metal powders including pure iron, carbonyl iron, Fe-Ni alloy (hereafter referred to as Permalloy), or Fe-Si-Aℓ alloy (hereafter referred to as Sendust) to which insulating binders such as sodium silicate or epoxy resin are added are compacted under pressure of 1-15 ton/cm² and then heat-treated to relieve compression stresses (Japan Society of Powder and Powder Metallurgy, Magnetic Materials (1970), The Nikkan Kogyo Shimbun, Ltd.).

JP-A-60-74602 discloses a dust core which is press-formed from metal magnetic powder obtained by using a water atomization method.

EP-A-0 088 992 discloses a method for manufacturing an object of soft-magnetic material by bonding together a mass of powder grains. These grains of iron and iron alloy powders have a particle size of 50 to 1000 µm and are coated with oxides of Fe, Si, Al and/or the like to a coating thickness of 0.01 to 0.5 µm, and are then subjected to isostatic pressing at a temperature of 600 to 900°C.

Pure iron powder cores are used in choke coils for switching power supplies at frequencies of 50 kHz or lower, transformers for ringing-choke-type power supply circuits, and noise suppressors in circuits in which low-frequency currents are superimposed.

Permalloy powder cores are used as cores for secondary-side smoothing chokes in switching power supplies in the frequency range of 100-150 kHz, and as noise-suppressors. Sendust powder cores can be used in the same frequency range as permalloy powder cores.

However, with recent requirements for severe control of high-frequency noise in electronic equipment, as well as for smaller and more compact equipment, powder cores of high permeability and low core loss are increasingly required. To manufacture powder cores, the powder particles are insulated by epoxy resin or sodium silicate to avoid direct contact between powder particles and decrease eddy current losses in the high-frequency region. Furthermore, pressing is used to increase density and obtain high permeability and low core loss.

In order to obtain high permeability, one needs to increase the packing density by high compacting pressure, but with conventional Sendust powder cores, the powder is extremely hard and resistant to plastic deformation, making high-pressure compacting difficult and markedly decreasing the life of dies.

Permalloy powder cores have higher permeability than pure iron powder cores and their high-frequency magnetic properties are excellent, but they are expensive and the adhesion of powder to the insulating layer is insufficient so that the insulation between particles breaks down, markedly degrading the magnetic properties in the high frequency region.

Therefore, an object of the present invention is to solve these problems by providing a process of manufacturing Fe-Si alloy powder cores and powder cores obtainable by such process which are inexpensive which have high permeability, excellent magnetic properties in the high frequency region and low core loss.

This object is achieved by a process according to Claim 1 and powder cores according to claim 3, respectively.

The objects and features of the present invention will become more apparent from the following detailed description taken in conjunction with the accompanying drawing, in which:

Figure 1 shows the variation of permeability with the frequency for powder cores of this invention along with other powder cores for comparison.

The inventors studied the effects on magnetic characteristics of interlayer insulation, powder compacting, powder composition and other factors which affect the magnetic properties in the high frequency region. As a result of this research, they found that Fe-Si alloy powders produced by water atomization form a stable oxide layer on the surface of the particles and have excellent compressibility, so that they may be manufactured into powder cores of high permeability and low core loss.

Specifically, the invention is an Fe-Si alloy powder core manufactured by compacting an alloy powder of an average particle diameter of 10-100 µm, produced by water atomization, in which the composition by weight of the alloy powder is 2-12% silicon, 0.05-0.95% oxygen and the balance being essentially iron.

More specifically, it is an Fe-Si alloy powder core in which the composition by weight of the alloy powder is 2-12% silicon, 0.05-0.95% oxygen, with an Aℓ, Cr and Ti content of less than 3% separately or combined, and the balance being essentially iron.

More specifically, it is a process of manufacturing Fe-Si alloy powder cores comprising the steps of adding an insulating binder to alloy powder of the above composition, compacting the resulting mixture and curing.

More specifically, it is a process of manufacturing Fe-Si alloy powder cores, comprising the above compacting step and curing step and a heat treatment step in which the compacted product is heat-treated in an inert atmosphere at a temperature between 500°C and 950°C.

The following is an explanation of the reasons for defining the invention in this manner.

The Si in the composition of the alloy powder of the invention is an essential component of this alloy, and if the Si content is less than 2%, electrical resistance will be decreased and eddy current losses in the high-frequency region will increase so that the desired permeability will not be obtained. If the Si content exceeds 12%, an intermetallic compound will be formed, making the powder hard and thus losing compressibility. The Si content is preferably between 3.0% and 7.5%, resulting in low magnetic anisotropy and magnetostriction.

Oxygen is vital to the formation of an insulating film on the surface of the powder, so if the oxygen content is less than 0.05%, a stable oxide layer will not be formed, and if greater than 0.95%, the oxide layer will become too thick, decreasing permeability and also decreasing the density of the green compacts. Therefore the oxygen content is in the range of 0.05-0.95%.

The Aℓ, Cr and Ti added to the essential components as optional components have the effect of further enhancing the stability of the insulating layer formed. If any of the elements are added individually or together in an amount exceeding 3%, the film will grow too thick, and the compressibility of the powder will be lowered, hence the 3% limitation.

The particle size of the powder greatly affects permeability and the quality of interparticle insulation. If the average particle size is less than 10 µm, the magnetic properties of the powder itself will be impaired, and a high packing density cannot be obtained so the desired level of permeability will not be attained. On the other hand, if the particle size exceeds 100 µm, excessive friction between particles will damage the insulating layer, so the magnetic properties in the high-frequency region will be impaired, hence the range of 10-100 µm.

Water atomization is a process of producing metal powder in which the raw material is melted and this molten metal is dropped through a tundish nozzle as a downward stream of molten metal of 2-20 mm in diameter. Water of high pressure, 50-800 kg/cm², is sprayed from an atomizing nozzle system onto this metal stream, which is disintegrated into fine droplets which solidify as powder (Metals Handbook Vol. 7, Page 25).

The water atomizing is easily controllable to obtain powder of the desired composition. In addition, since the metal is quenched by water, the particles are irregular in shape, giving the powder excellent compressibility and a low demagnetization factor. In addition, since the metal is oxidized by the water, the thickness of the oxide layer, and hence the oxygen content of the alloy powder, may be controlled by altering the atmosphere during atomization or altering the dissolved oxygen content of the water. Thus powder suited to the powder core of the invention may be produced.

In water atomization, an atomizing nozzle is provided on the inside top of an atomizing chamber. Molten metal is dropped as a fine stream from the top of the chamber and atomized as high-pressure water from the nozzle strikes the metal stream. Thus if atomization is carried out in air as the atmosphere within the chamber, in the case of iron powder, the amount of oxygen of the powder will reach a level of 3-5%. If the chamber atmosphere is replaced by nitrogen, argon or another inert gas and the inside of the chamber is filled with water to rapidly quench the drops of atomized metal, the oxygen content of the iron powder can be decreased to about 1%. Furthermore, if Ar, N₂ or another gas is bubbled through the water used in atomizing and vacuum treatment employed to reduce dissolved oxygen in the water prior to atomization, the oxygen content of the iron powder can be decreased to less than 0.1%. The dissolved oxygen content of the water can be altered to control the oxygen content of the powder within the range of 0.05-0.95%.

Water-atomized Fe-Si alloy powder produced in this manner will have an average particle size of 10-100 µm after sieving. An insulating binder, typically sodium silicate, epoxy resin or, if heat treatment will be carried out, a heat-resistant resin such as silicone resin will be added in the amount of 1-10% by weight and mixed. Next, compacting under a pressure of 1-15 ton/cm² will be used to make compacts of the desired shape, and then hardening treatment and, if necessary, heat treatment will be carried out. Finally, an insulating coating is painted onto the surface and the powder core is manufactured.

After adding insulating binder to Fe-Si alloy particles and compacting, the compacts are hardened by a hardening treatment in which they are heated to 100-300°C, depending on the type of insulating binder and the application for the powder core. When heat treatment is carried out as described hereafter, the curing step may be omitted.

Note that in order to improve the adhesion of the resin or the like used as the insulating binder, it is preferable to treat the surface of the Fe-Si alloy powder used as the raw material with a Ti- or Si-based organometallic coupling agent.

While Fe-Si alloy powder can be used in this manner to manufacture powder cores having excellent electromagnetic properties, the electromagnetic properties may be further improved by heat-treating the compacted cores.

Heat treatment is effective when carried out at a temperature between 500°C and 950°C in an inert atmosphere of nitrogen or argon. As to the environment, ordinary air cannot be used because the alloy powder would oxidize, and hydrogen, cracked ammonia gas or other reducing environments alter the characteristics of the oxide layer. Thus a nitrogen or argon atmosphere is preferable.

As to the temperature, the relief of compacting stress is difficult at less than 500°C, while if 950°C is exceeded, the insulating layer breaks down and the powder particles are sintered together and the magnetic properties in the high-frequency region deteriorate. Thus heat treatment at a temperature between 500°C and 950°C relieves stress in the core and causes the structure to change to improve electromagnetic properties by forming a superlattice structure.

As to the heat treatment time, the time should generally be longer at lower temperature and shorter at high temperature, but nevertheless it should be 1-20 hours, preferably 1-5 hours.

Fe-Si alloy powders of various compositions as listed in Table 1 were fabricated and sieved to the desired average particle size.

The oxygen content of the alloy powder was altered by using Ar gas as the atomizing atmosphere and by bubbling Ar gas through the cooling water and atomizing water.

To these powders was added 1.5% by weight of epoxy resin and then the mixture was pressed at pressure of 8 ton/cm² into a ring of outside diameter 20 mm, inside diameter 12 mm and height 8 mm. Hardening treatment was then carried out at 150°C for 2 hours, after which an impedance meter was used to measure the variation of permeability with frequency.

Before heat treatment was carried out, sodium silicate was added to the Fe-Si alloy powder in an amount of 1.0% by weight, and the mixture was pressed at a pressure of 8 ton/cm².

The heat treatment was carried out in an argon atmosphere.

The results of an evaluation of characteristics of the powder cores are listed in Table 1.

In the table, the notation µe10K indicates the permeability at a frequency of 10 kHz, while µe10M/µe10K indicates the ratio of permeability at 10 MHz to permeability at 10 kHz, and this is taken as an indication of the magnetic properties in the high-frequency region.

As is apparent from Table 1, the oxygen content of cores 1-9 of the invention is in the range 0.05-0.95%, the average particle size is in the range 10-100 µm and each core exhibits high permeability at 10 kHz of 70 or greater. Of particular note is the high-frequency properties in that the permeability at 10 MHz is the same or greater than the permeability at 10 kHz.

In particular, the cores of the invention which had been heat treated, namely cores 8-13, maintained a high permeability even up to the high-frequency region.

Of the cores for comparison, the Sendust powder core 4, the pure iron powder core 5 and the Permalloy powder core 6 each have a higher permeability at 10 kHz than cores 1-5 of the invention, but a lower permeability at 10 MHz, so their high-frequency properties are inferior.

In addition, core 1 for comparison is made from powder of such small particle size that the magnetism of the powder itself is poor, while the particle size of core 2 for comparison is so large that the insulating performance is inferior in the high-frequency range.

In core 3 for comparison, in which the Si content exceeds 12%, the powder is so hard that the packing density is insufficient and the permeability at 10 kHz is low.

In core 7 for comparison, the gas atomization by which the powder was produced caused the particles to be spherically-shaped and thus the demagnetization factor is high and the permeability low. Core 8 for comparison has a thick oxide layer so its permeability is low. Core 9 for comparison was subjected to high-temperature annealing, so the powder became sintered, thus increasing permeability in the low-frequency range but giving inferior properties in high-frequency region. Core 10 for comparison is made from carbonyl iron powder so while the high-frequency properties is good, the absolute value of the permeability is low.

Figure 1 shows the variation of permeability with frequency for several cores in Table 1 fabricated by the same steps as above. The cores on the graph are cores 2 and 8 of the invention and cores 4, 5 and 10 for comparison. Core 2 of the invention exhibits high permeability even at frequencies above 10 MHz, while the permeability of the cores for comparison begins to drop off at around 1 MHz.

Thus it is evident that the cores of the invention have good high-frequency magnetic properties.

## Claims

1. A process of manufacturing an Fe-Si alloy powder core comprising the following steps:
a) producing an alloy powder comprising by weight 2-12% Si, 0.05-0.95% 0 and optionally less than 3% Al, Cr and/or Ti with the balance of Fe by water atomization in which a stream of molten metal is poured into an atomization tank and sprayed with high pressure water for atomizing the metal stream to obtain irregularly shaped alloy powder particles of an average particle diameter of 10-100 µm wherein the atmosphere of the atomization tank and/or the dissolved oxygen content of the high-pressure water is adjusted for controlling the oxygen content of the alloy powder,
b) adding an insulating binder to the alloy powder,
c) forming the resulting mixture and
d) subjecting the formed mixture to a hardening treatment.

2. A process according to claim 1, wherein the formed mixture is subjected to heat treatment in an inert atmosphere at a temperature in the range of 500-950 °C.

3. An Fe-Si alloy powder core obtainable by a process according to claim 1 or 2.

## Patentansprüche

1. Verfahren zur Herstellung eines Kerns aus Fe-Si-Legierungspulver mit den folgenden Schritten:
a) Herstellen eines Legierungspulvers mit 2 bis 12 Gew.-% Si, 0,05 bis 0,95 Gew.-% O und wahlweise weniger als 3 Gew.-% Al, Cr und/oder Ti, wobei der Rest Eisen ist, durch Wasserverdüsung, bei der ein Metallschmelzstrom in einen Verdüsungsbehälter gegossen und mit Wasser unter hohem Druck zum Verdüsen des Metallstroms besprüht wird, um unregelmäßig geformte Legierungspulverteilchen mit einer durchschnittlichen Teilchengröße von 10 bis 100 µm zu erhalten, wobei die Atmosphäre des Verdüsungsbehälters und/oder der Gelöstsauerstoffgehalt des unter hohem Druck stehenden Wassers zum Steuern des Sauerstoffgehalts des Legierungspulvers eingestellt wird,
b) Zufügen eines Isolierbindemittels zu dem Legierungspulver,
c) Formen der resultierenden Mischung und
d) Durchführen einer Härtungsbehandlung der geformten Mischung.

2. Verfahren nach Anspruch 1, wobei die geformte Mischung einer Wärmebehandlung in einer Inertatmosphäre bei einer Temperatur im Bereich von 500 bis 950 °C unterzogen wird.

3. Kern aus Fe-Si-Legierungspulver, der durch ein Verfahren gemäß Anspruch 1 oder 2 erhältlich ist.

## Revendications

1. Un procédé de fabrication d'un noyau en poudre d'un alliage Fe-Si comprenant les étapes suivantes :
a) production d'une poudre d'alliage comprenant, en poids, 2-12% de Si, 0,05-0,95 % de 0 et optionnellement moins de 3% de Al, de Cr et/ou de Ti, avec le reste étant du fer, par une atomisation à l'eau dans laquelle un flux de métal fondu est versé dans un réservoir d'atomisation et est aspergé d'eau à haute pression pour atomiser le flux de métal afin d'obtenir des particules de poudre d'alliage de forme irrégulière d'un diamètre moyen des particules de 10-100µm, dans laquelle l'atmosphère du réservoir d'atomisation et/ou la teneur en oxygène dissous de l'eau à haute pression sont ajustées pour contrôler la teneur en oxygène de la poudre d'alliage,
b) addition d'un liant isolant à la poudre d'alliage,
c) formage du mélange résultant et
d) soumission du mélange formé à un traitement de durcissement.

2. Un procédé selon la revendication 1, dans lequel le mélange formé est soumis à un traitement thermique dans une atmosphère inerte à une température dans la plage de 500-950°C.

3. Un noyau en poudre d'un alliage Fe-Si pouvant être obtenu par un procédé selon la revendication 1 ou 2.
